



US006652392B2

(12) **United States Patent**  
Higuchi et al.

(10) **Patent No.:** US 6,652,392 B2  
(45) **Date of Patent:** Nov. 25, 2003

(54) **MULTI-PIECE SOLID GOLF BALL**

(75) Inventors: **Hiroshi Higuchi**, Chichibu (JP);  
**Hirotaka Shimosaka**, Chichibu (JP);  
**Atsuki Kasashima**, Chichibu (JP);  
**Junji Umezawa**, Chichibu (JP)

(73) Assignee: **Bridgestone Sports Co., Ltd.**, Tokyo (JP)

(\*) Notice: Subject to any disclaimer, the term of this patent is extended or adjusted under 35 U.S.C. 154(b) by 0 days.

(21) Appl. No.: **10/022,868**

(22) Filed: **Dec. 20, 2001**

(65) **Prior Publication Data**

US 2002/0119832 A1 Aug. 29, 2002

(30) **Foreign Application Priority Data**

Dec. 22, 2000 (JP) ..... 2000-389794

(51) **Int. Cl.**<sup>7</sup> ..... **A63B 37/06**

(52) **U.S. Cl.** ..... **473/374**

(58) **Field of Search** ..... 473/351, 370, 473/373, 374, 376, 378

(56) **References Cited**

## U.S. PATENT DOCUMENTS

- 4,919,434 A \* 4/1990 Saito ..... 473/373  
5,314,187 A 5/1994 Proudfit  
5,553,852 A 9/1996 Higuchi et al.  
5,779,562 A 7/1998 Melvin et al.  
5,779,563 A 7/1998 Yamagishi et al.  
5,890,974 A \* 4/1999 Stiefel et al. ..... 473/384  
5,899,822 A 5/1999 Yamagishi et al.

|                |         |                              |
|----------------|---------|------------------------------|
| 5,906,551 A    | 5/1999  | Kasashima et al.             |
| 6,015,356 A    | 1/2000  | Sullivan et al.              |
| 6,142,885 A    | 11/2000 | Umezawa et al.               |
| 6,174,247 B1   | 1/2001  | Higuchi et al.               |
| 6,267,692 B1 * | 7/2001  | Higuchi et al. ..... 473/365 |

## FOREIGN PATENT DOCUMENTS

|    |              |                           |
|----|--------------|---------------------------|
| EP | 0 846 478 A1 | 6/1998                    |
| EP | 0 895 791 A1 | 2/1999                    |
| GB | 2278609 A    | 7/1994                    |
| JP | 11-104272    | * 4/1999 ..... A63B/37/00 |
| JP | 2000-157647  | 6/2000                    |

## OTHER PUBLICATIONS

European Search Report for EP 01 31 0744, Apr. 28, 2003.

\* cited by examiner

*Primary Examiner*—Mark S. Graham

*Assistant Examiner*—Raeann Gorden

(74) *Attorney, Agent, or Firm*—Sughrue Mion, PLLC

(57) **ABSTRACT**

In a multi-piece solid golf ball comprising an elastic solid core and a resin cover, the cover includes at least an inner layer and an outer layer, the solid core undergoes a deflection of 1.1–4.0 mm under a load of 294 N, the cover inner and outer layers have a Shore D hardness of 45–70 and 35–55, respectively. The ball is provided with a multiplicity of dimples which are substantially uniformly arranged such that a great circle which does not intersect with the dimples is absent. The ball exhibits consistent flight performance when hit with a driver, suppresses reduction of spin when hit in the wet state with a short iron, and offers stable ready-to-strike conditions, flight performance and spin performance under any conditions covering from the fairway to the putting green.

14 Claims, 4 Drawing Sheets



**FIG.1**

**FIG.2****FIG.3**

**FIG.4****FIG.5**

**FIG.6****FIG.7**

## MULTI-PIECE SOLID GOLF BALL

This invention relates to a dimpled multi-piece solid golf ball comprising an elastic solid core and a resin cover of a plurality of layers enclosing the solid core, and more particularly, to a dimpled multi-piece solid golf ball which ensures consistent flight and has improved controllability in that it suppresses substantial reduction of spin when hit in the wet state with a short iron. As used herein, the term "wet state" refers to the state of a golf course in rain weather, and the term "dry state" refers to the state of a golf course in fine weather.

## BACKGROUND OF THE INVENTION

One of known solid golf balls has the structure in which a rubbery elastic solid core is enclosed with a cover of relatively hard ionomer resin characterized by good external damage prevention such as cut resistance and abrasion resistance. A multiplicity of dimples are arranged on the outer surface of the cover so as to achieve a uniform distribution.

Molds used to mold the cover about the core are generally of the two-division type, that is, constructed from a pair of mold halves which are mated along a parting plane to define a spherical cavity. The parting plane is located in register with the equator of the spherical cavity. Therefore, for the convenience of mold manufacture, a mold in which the placement of dimples (exactly stated, dimple-forming protrusions) at positions that lie in the parting plane is avoided is generally used. This destroys the uniformity of dimple arrangement about the overall ball including the proximity of the equator, even if the uniform arrangement of dimples is accomplished on each of the hemispheres divided along the equator.

On account of such a non-uniform arrangement or non-uniform dispersion of dimples, the aerodynamic effect of dimples exerted when the ball is hit differs with the spin direction, that is, between the case where the ball spins about an axis passing the center of the ball and parallel to the equator plane and the case where the ball spins about an axis passing the opposite poles of the ball and perpendicular to the equator plane. This causes variations in the flight direction and distance of the ball when hit with a club which is designed to gain distance, as typified by a driver. The ball lacks flight consistency.

In connection with the material aspect and physical properties of the cover, the golf ball has the following problem. The ball performs well in the dry state or fine weather in that it travels a satisfactory distance when hit with a driver and receives a requisite spin when hit with an iron which demands controllability to the ball. In the wet state or rain weather, however, the ball becomes less susceptible to spin and therefore, becomes less controllable when hit with an iron club. In particular, the spin susceptibility of the ball when hit with a short iron having a loft of an 8-iron or greater is degraded. As a result, the ball will travel a longer distance than intended or will not stop immediately on the green.

In these regards, the prior art golf balls are not fully satisfactory to professional and low-handicap golfers. It is desired to overcome the above problems.

## SUMMARY OF THE INVENTION

Therefore, an object of the invention is to provide a dimpled multi-piece solid golf ball comprising an elastic solid core and a resin cover of a plurality of layers, which

ball is improved for short iron shots in that the percent retention of the spin the ball receives when hit with the short iron in the wet state from the spin the ball receives when hit with the short iron in the dry state is high and which ball exhibits flight consistency when hit with a club designed to gain distance, as typified by a driver.

According to the invention, there is provided a multi-piece solid golf ball comprising an elastic solid core and a resin cover enclosing the solid core, the cover being composed of a plurality of layers including an inner layer disposed adjacent to the solid core and an outer layer disposed radially outside the inner layer. The solid core has a hardness corresponding to a deflection of at least 1.1 mm under an applied load of 294 N (30 kgf), the cover inner layer has a Shore D hardness of 45 to 70, and the cover outer layer has a Shore D hardness of 35 to 55. The ball is provided on its surface with a multiplicity of dimples which are substantially uniformly arranged on the ball surface such that a great circle which does not intersect with the dimples is absent.

In a preferred embodiment, provided that the ball receives a spin rate  $S_1$  (rpm) in the dry state and a spin rate  $S_2$  (rpm) in the wet state when hit with a short iron having a loft of an 8-iron or greater, the percent spin retention given by  $(S_2/S_1) \times 100$  is at least 47%.

Preferably the cover outer layer is softer than the cover inner layer. Also preferably, the cover inner layer has a Shore D hardness A and the cover outer layer has a Shore D hardness B, and A and B satisfy the relationship:  $A \times B \geq 2300$ . Preferably, the cover outer layer is formed mainly of a thermoplastic polyurethane elastomer, thermosetting polyurethane elastomer, polyester elastomer or a mixture thereof. More preferably, the cover outer layer is formed mainly of a thermoplastic polyurethane elastomer obtained using an aromatic or aliphatic diisocyanate, or the reaction product of a thermoplastic polyurethane elastomer with an isocyanate compound. Also preferably, the cover inner layer is formed mainly of an ionomer resin. An adhesive layer may intervene between the cover inner and outer layers.

Preferably, the core has a specific gravity of 1.0 to 1.3, the cover inner layer has a specific gravity of 0.8 to 1.4, and the cover outer layer has a specific gravity of 0.9 to 1.3.

The invention ensures the manufacture of a seamless golf ball on the surface of which dimples are substantially uniformly arranged so that a great circle which does not intersect with the dimples is absent. The flight distance is consistent whether the ball is hit with a driver or an iron. The spin susceptibility of the ball when hit with a short iron having a loft of an 8-iron or greater is not reduced in the dry state or fine weather, nor is noticeably reduced even in the wet state or rain weather. Then the ball travels a distance as intended, immediately stops on the green, and is easy to control. Since the ball offers stable ready-to-strike conditions, flight performance and spin performance under any conditions covering from the fairway (driver) to the putting green (iron), it is a high-performance solid golf ball suited for professional and amateur low-handicap golfers to play with.

## BRIEF DESCRIPTION OF THE DRAWING

FIG. 1 is a cross-sectional view of a multi-piece solid golf ball according to one embodiment of the invention.

FIG. 2 is a side view showing the dimple arrangement pattern on the golf balls of Examples 1 and 3.

FIG. 3 is a side view showing the dimple arrangement pattern on the golf ball of Example 2.

FIG. 4 is a side view showing the dimple arrangement pattern on the golf ball of Example 4.

FIG. 5 is a side view showing the dimple arrangement pattern on the golf balls of Comparative Examples 1 and 3.

FIG. 6 is a side view showing the dimple arrangement pattern on the golf ball of Comparative Example 4.

FIG. 7 is a side view showing the dimple arrangement pattern on the golf ball of Comparative Example 5.

#### DESCRIPTION OF THE PREFERRED EMBODIMENT

The multi-piece solid golf ball of the invention is embodied in FIG. 1 as comprising a solid core 1, a cover inner layer 2 enclosing the core 1, and a cover outer layer 3 enclosing the inner layer 2, all in a concentric manner. The cover inner layer 2 is a single layer in the illustrated embodiment although it may be composed of two or more layers. It is noted that the cover is provided on the outer surface with a multiplicity of dimples D.

The solid core 1 is preferably formed of a rubber composition, which is preferably based on polybutadiene. The preferred polybutadiene is cis-1,4-polybutadiene having at least 40% of cis configuration. In the base rubber, polybutadiene is compounded with another rubber such as natural rubber, polyisoprene rubber or styrene-butadiene rubber if desired. Increasing the rubber content leads to golf balls with improved rebound.

In the rubber composition, there may be blended a crosslinking agent, for example, zinc and magnesium salts of unsaturated fatty acids such as zinc dimethacrylate and zinc diacrylate and esters such as trimethylpropane methacrylate. Zinc diacrylate is especially preferred. The crosslinking agent is preferably used in an amount of at least about 10 parts and up to about 50 parts by weight, and especially at least about 20 parts and up to about 45 parts by weight per 100 parts by weight of the base rubber.

A vulcanizing agent is generally blended in the rubber composition. It is recommended that the vulcanizing agent include a peroxide having a 1-minute half-life temperature of not higher than 155° C., the content of the peroxide being at least 30% by weight, and especially at least 40% by weight, of the overall vulcanizing agent. No particular upper limit is imposed on the content of peroxide, although this content is preferably not more than 70% by weight. Examples of suitable peroxides include commercially available products such as Perhexa 3M (manufactured by NOF Corp.). The amount of vulcanizing agent blended in the rubber composition is preferably set at about 0.6 to about 2 parts by weight per 100 parts by weight of the base rubber.

If necessary, other suitable ingredients may also be added to the rubber composition, including antioxidants and specific gravity-adjusting fillers such as zinc oxide and barium sulfate.

The solid core can be prepared from the above-described rubber composition. For example, after the components are kneaded in a conventional mixer such as a Banbury mixer or roll mill, the kneaded material is compression or injection molded in a core-forming mold where it is heated to a sufficient temperature for the crosslinking and vulcanizing agents to work, thereby effecting vulcanization or cure. In one example where dicumyl peroxide is used as the vulcanizing agent and zinc diacrylate used as the crosslinking agent, the material is heated at about 130 to about 170° C. for about 10 to 40 minutes, and especially at about 150 to about 160° C. for about 12 to 20 minutes.

As noted above, the solid core is prepared from the rubber composition by well-known molding and vulcanizing or curing techniques. The solid core typically has a diameter of at least 30 mm, more preferably at least 33 mm, even more preferably at least 35 mm and up to 40 mm, more preferably up to 39 mm, even more preferably up to 38 mm.

With respect to the hardness, the solid core should undergo a deflection under an applied load of 294 N (30 kgf) of at least 1.1 mm, preferably at least 1.2 mm, more preferably at least 1.4 mm, even more preferably at least 1.5 mm and preferably up to 4.0 mm, more preferably up to 3.5 mm, even more preferably up to 3.0 mm, further preferably up to 2.5 mm, most preferably up to 2.3 mm. If the deflection of the core under an applied load of 294 N (30 kgf) is less than 1.1 mm, the feel of the ball when hit becomes undesirably hard. Too large a deflection may lead to losses of resilience and durability. The core has a hardness (JIS-C hardness) distribution in cross section which may be leveled or graded between the center and the outer surface or may locally vary (local hardness difference).

Preferably the solid core has a specific gravity of at least 1.0, more preferably at least 1.05, even more preferably at least 1.1 and up to 1.3, more preferably up to 1.25, even more preferably up to 1.2.

The solid core may have either a single-layer structure formed of one material or a multi-layer structure of two or more concentric layers of different materials.

According to the invention, the solid core is enclosed with a resin cover consisting of a plurality of layers, typically two layers, inner layer 2 and outer layer 3 as shown in FIG. 1. The cover inner layer has a Shore D hardness of 45 to 70, and the cover outer layer has a Shore D hardness of 35 to 55. Preferably the cover outer layer is made softer than the cover inner layer.

The cover inner layer is preferably formed of a material based on a resin component such as an ionomer resin or a blend of an ionomer resin with an olefin elastomer. Also useful are blends of an ionomer resin with a polyester elastomer, ionomer resins having an increased degree of neutralization, and ionomer resins having an increased acid content.

The blend of an ionomer resin with an olefin elastomer exhibits better properties (e.g., hitting feel and rebound) which cannot be arrived at using the components alone. Examples of the olefin elastomer include linear low-density polyethylene, low-density polyethylene, high-density polyethylene, polypropylene, rubber-reinforced olefin polymers, flexomers, plastomers, thermoplastic elastomers containing acid-modified ones (e.g., styrene base block copolymers and hydrogenated polybutadiene-ethylene-propylene rubber), dynamically vulcanized elastomers, ethylene acrylate, and ethylene vinyl acetate. Commercially available products include HPR from Dupont-Mitsui Polymers Co., Ltd. and Dynaron from JSR Corporation. The weight ratio of the ionomer resin to the olefin elastomer is preferably from 40:60 to 95:5, more preferably from 45:55 to 90:10, even more preferably from 48:52 to 88:12, and most preferably from 55:45 to 85:15. Too low a proportion of the olefin elastomer may often lead to a hard feel whereas too high a proportion thereof may lead to a decline of resilience.

The ionomer resins which can be used herein are of the neutralized type with such ions as Zn, Mg, Na and Li. An ionomer resin material is recommended comprising 5 to 100%, more preferably 10 to 80%, most preferably 15 to 70% by weight of a Zn or Mg ion-neutralized type ionomer

resin which is relatively flexible and resilient. The ionomer resin may be blended with another polymer as long as it does not compromise the benefits of the invention.

The cover inner layer may also be formed of a blend of an ionomer resin with a polyester elastomer. The weight ratio of the ionomer resin to the polyester elastomer is preferably from 40:60 to 95:5, more preferably from 45:55 to 90:10, even more preferably from 48:52 to 88:12, and most preferably from 55:45 to 85:15. Too low a proportion of the polyester elastomer may often lead to a hard feel whereas too high a proportion thereof may lead to a decline of resilience.

Also, the cover inner layer may be formed of a material comprising an ionomer resin, a fatty acid or derivative thereof having a molecular weight of at least 280, and a basic inorganic metal compound capable of neutralizing acid groups in the foregoing components, which are heated and mixed so that the degree of neutralization of acid groups on the ionomer resin is increased. Moreover, an ionomer resin having an increased acid content, such as Himilan AM7317 and AM7318 from Dupont-Mitsui Polymers Co., Ltd. may be used to form the cover inner layer.

It is preferred that the material of which the cover inner layer is made contain less than about 30%, especially 1 to 20% by weight of an inorganic filler such as zinc oxide, barium sulfate and titanium dioxide.

The cover inner layer should have a Shore D hardness of at least 45, preferably at least 50, more preferably at least 53, even more preferably at least 55, and most preferably at least 57 and up to 70, preferably up to 68, more preferably up to 66, even more preferably up to 64, and most preferably up to 62. The cover inner layer with too low a Shore D hardness provides the ball with less rebound whereas too high a Shore D hardness gives a hard feel.

The cover inner layer should preferably have a specific gravity of at least 0.8, more preferably at least 0.9, even more preferably at least 0.92 and most preferably at least 0.93 and up to 1.4, more preferably up to 1.16, even more preferably up to 1.1 and most preferably up to 1.05.

The cover inner layer preferably has a gage or radial thickness of at least 0.5 mm, more preferably at least 0.7 mm, even more preferably at least 0.9 mm, most preferably at least 1.1 mm and up to 3.0 mm, more preferably up to 2.5 mm, even more preferably up to 2.0 mm.

The cover outer layer **3** is preferably formed mainly of a thermoplastic polyurethane elastomer, thermosetting polyurethane elastomer, polyester elastomer or a mixture of any, although the material is not limited thereto. Also useful are polyamide elastomers, ionomer resins, blends of polyester elastomer and ionomer resin in a weight ratio between 100/0 and 60/40, compositions based on a thermoplastic polyurethane elastomer prepared using an aromatic or aliphatic isocyanate, and compositions based on the reaction product of the thermoplastic polyurethane elastomer with an isocyanate compound.

The thermoplastic polyurethane elastomer has a molecular structure including soft segments of a high molecular weight polyol and hard segments constructed of a mono-molecular chain extender and a diisocyanate. The high molecular weight polyol compounds used herein include, though are not limited thereto, polyester polyols, polyether polyols, copolyester polyols, and polycarbonate polyols. The polyester polyols include polycaprolactone glycol, poly(ethylene-1,4-adipate) glycol, and poly(butylene-1,4-adipate) glycol. Typical of the copolyester polyols is poly(diethylene glycol adipate) glycol. One exemplary

polycarbonate polyol is (hexanediol-1,6-carbonate) glycol. Polyoxytetramethylene glycol is typical of the polyether polyols. These polyols have a number average molecular weight of about 600 to 5,000, preferably about 1,000 to 3,000. The chain extender used herein may be any of commonly used polyhydric alcohols and amines. Examples include 1,4-butylene glycol, 1,2-ethylene glycol, 1,3-propylene glycol, 1,6-hexylene glycol, 1,3-butylene glycol, dicyclohexylmethane diamine (hydrogenated MDA), and isophorone diamine (IPDA). The diisocyanates used herein are preferably aliphatic diisocyanates and aromatic diisocyanates. Exemplary aliphatic diisocyanates include hexamethylene diisocyanate (HDI), 2,2,4- or 2,4,4-trimethylhexamethylene diisocyanate (TMDI), and lysine diisocyanate (LDI). Exemplary aromatic diisocyanates include 2,4-toluene diisocyanate, 2,6-toluene diisocyanate, and 4,4-diphenylmethane diisocyanate. Of these, aliphatic diisocyanates are preferred from the standpoint of the cover's yellowing resistance, and HDI is most preferable because of compatibility in blending with other resins.

Of the thermoplastic polyurethane elastomers, those elastomers which on viscoelasticity measurement, exhibit a  $\tan\delta$  peak temperature of  $-15^{\circ}\text{C}$ . or lower, more preferably  $-16^{\circ}\text{C}$ . or lower, with the lower limit being  $-50^{\circ}\text{C}$ . or higher, are preferred from the flexibility and resilience standpoint. Such thermoplastic polyurethane elastomers are commercially available under the trade name of Pandex T7298 ( $-20^{\circ}\text{C}$ ), T7295 ( $-26^{\circ}\text{C}$ ), and T7890 ( $-30^{\circ}\text{C}$ ) from Bayer DIC Polymer Co., Ltd. in which the diisocyanate is aliphatic. It is noted that the temperature in parentheses indicates the  $\tan\delta$  peak temperature.

As the cover outer layer material, the reaction product of the above-described thermoplastic polyurethane elastomer with an isocyanate compound may also be used because it can further improve the surface durability of the cover against iron shots.

The isocyanate compound used herein may be any of isocyanate compounds used in conventional polyurethanes. Exemplary aromatic isocyanate compounds include 2,4-toluene diisocyanate, 2,6-toluene diisocyanate or a mixture thereof, 4,4-diphenylmethane diisocyanate, m-phenylene diisocyanate, and 4,4'-biphenyl diisocyanate. Hydrogenated products of these aromatic isocyanate compounds, for example, dicyclohexylmethane diisocyanate are also useful. Also included are aliphatic isocyanates such as tetramethylene diisocyanate, hexamethylene diisocyanate (HDI) and octamethylene diisocyanate as well as alicyclic diisocyanates such as xylene diisocyanate. Other useful examples include blocked isocyanate compounds obtained by reacting a compound having at least two isocyanate groups at the end with a compound having active hydrogen, and uretidione forms resulting from isocyanate dimerization.

An appropriate amount of the isocyanate compound used is generally at least 0.1 part, preferably at least 0.2 part, more preferably at least 0.3 part by weight and up to 10 parts, preferably up to 5 parts, more preferably up to 3 parts by weight, per 100 parts by weight of the thermoplastic polyurethane elastomer. Too small an amount of the isocyanate compound may fail to induce sufficient crosslinking reaction, with little improvements in physical properties being observed. Too large an amount may give rise to several problems including substantial discoloration by aging, heat and ultraviolet radiation, the loss of thermoplasticity and a decline of resilience.

The thermosetting polyurethane of which the cover outer layer is made is obtained from a polyisocyanate such as

2,4-toluene diisocyanate (TDI), methylenebis(4-cyclohexyl isocyanate) (HMDI), 4,4'-diphenylmethane diisocyanate (MDI) or 3,3'-dimethyl-4,4'-biphenylene diisocyanate (TODI) and a polyol which will cure with a polyamine such as methylene dianiline (MDA), a trihydric glycol such as trimethylol propane or a tetrahydric glycol such as N,N,N',N'-tetrakis(2-hydroxypropyl)ethylene diamine.

Preferred polyether polyols are polytetramethylene ether glycol, poly(oxypropylene) glycol and polybutadiene glycol. Preferred polyester polyols are polyethylene adipate glycol, polyethylene propylene adipate glycol and polybutylene adipate glycol. Preferred polylactone polyols are diethylene glycol-initiated caprolactone, 1,4-butane-diol-initiated caprolactone, trimethylol propane-initiated caprolactone and neopentyl glycol-initiated caprolactone. Of these polyols, preferred are polytetramethylene ether glycol, polyethylene adipate glycol, polybutylene adipate glycol and diethylene glycol-initiated caprolactone.

A suitable curing agent is selected from slow-reactive polyamines such as 3,5-dimethylthio-2,4-toluenediamine, 3,5-dimethylthio-2,6-toluenediamine, N,N'-dialkyldiaminodiphenylmethanes, trimethylene glycol di-p-aminobenzoate, polytetramethylene oxide di-p-aminobenzoate, dihydric glycols, and mixtures thereof. It is noted that 3,5-dimethylthio-2,4-toluenediamine and 3,5-dimethylthio-2,6-toluenediamine are isomers and commercially available under the trade name of ETHACURE® 300 from Ethyl Corporation; trimethylene glycol di-p-aminobenzoate and polytetra-methylene oxide di-p-aminobenzoate are available under the trade name of POLACURE 740M and POLAMINES, respectively, from Polaroid; and N,N'-dialkyldiaminodiphenylmethane is available under the trade name of UNILINK® from UOP.

Preferred glycol is PTMEG or poly(tetramethylene ether) glycol.

Preferred dihydric glycols are 1,4-butanediol, 1,3-butanediol, 2,3-butanediol, 2,3-dimethyl-2,3-butanediol, dipropylene glycol and ethylene glycol. The dihydric glycols are essentially slow reactive.

As noted above, the thermosetting polyurethanes can be prepared from a number of commercially available aromatic, aliphatic and alicyclic diisocyanates and polyisocyanates.

The thermoplastic polyester elastomers of which the cover outer layer is made are multi-block copolymers of the polyether ester family which are synthesized from terephthalic acid, 1,4-butanediol, polytetramethylene glycol (PTMG) and polypropylene glycol (PPG) and therefore, comprise hard segments of polybutylene terephthalate (PBT) and soft segments of polytetramethylene glycol (PTMG) and polypropylene glycol (PPG). They are commercially available as Hytrel 3078, 4047, G3548W, 4767 and 5577 from Dupont Toray Co., Ltd.

The polyamide elastomers of which the cover outer layer is made are multi-block copolymers of the polyamide family which comprise hard segments of a nylon oligomer such as nylon 6, 11 or 12 and soft segments of polytetramethylene glycol (PTMG) or polypropylene glycol (PPG). They are commercially available as Pebax 2533, 3533 and 4033 from Elf Atochem.

Useful ionomer resins are those customarily used as the cover stock for solid golf balls. Such ionomer resins are commercially available, for example, under the trade name of Himilan 1855 from Dupont Mitsui Polymers Co., Ltd., and Surlyn 8120, 8320 and 6320 from E. I. Dupont. A mixture of two or more ionomer resins is also useful.

These cover materials may be used alone or in admixture. Blends of each of the foregoing resins with an ionomer resin are also useful. If necessary, well-known additives such as pigments, dispersants, antioxidants, UV absorbers and plasticizers may be blended in the cover material.

The cover outer layer should have a Shore D hardness of at least 35, preferably at least 38, more preferably at least 41, even more preferably at least 44, most preferably at least 47 and up to 55, preferably up to 53, more preferably up to 51, even more preferably up to 50, most preferably up to 49. The Shore D hardness of the cover outer layer should preferably be lower than that of the cover inner layer. The cover outer layer with too low a Shore D hardness has a propensity to receive too much spin, resulting in a reduced flight distance. Too high a Shore D hardness suppresses spin to an extremely low rate to decline controllability and reduces the spin consistency between dry and wet state shots.

The cover outer layer should preferably have a specific gravity of at least 0.9, more preferably at least 0.95, even more preferably at least 1.0 and most preferably at least 1.05 and up to 1.3, more preferably up to 1.25, even more preferably up to 1.22 and most preferably up to 1.19. The cover outer layer preferably has a gage or radial thickness of at least 0.5 mm, more preferably at least 0.7 mm, even more preferably at least 0.9 mm and most preferably at least 1.1 mm and up to 2.5 mm, more preferably up to 2.3 mm, even more preferably up to 2.0 mm.

In one preferred embodiment, provided that the cover inner layer has a Shore D hardness A and the cover outer layer has a Shore D hardness B, A and B satisfy the relationship:  $A \times B \geq 2300$ , more preferably  $A \times B \geq 2500$ , and most preferably  $A \times B \geq 2800$ . If  $A \times B < 2300$ , then problems arise like too much spin and reduced flight distance.

Any desired technique may be used to form the cover inner and outer layers. Use may be made of conventional injection molding and compression molding techniques.

In one preferred embodiment, an adhesive layer intervenes between the cover inner layer and the cover outer layer for the purpose of improving the durability against strikes. As the adhesive, epoxy resin base adhesives, vinyl resin base adhesives, and rubber base adhesives may be used although urethane resin base adhesives and chlorinated polyolefin base adhesives are preferred.

Dispersion coating may be used to form the adhesive layer. The type of emulsion which is used in dispersion coating is not critical. The resin powder used in preparing the emulsion may be either thermoplastic resin powder or thermosetting resin powder. Exemplary resins are vinyl acetate resins, vinyl acetate copolymer resins, EVA (ethylene-vinyl acetate copolymer resins), acrylate (co) polymer resins, epoxy resins, thermosetting urethane resins, and thermoplastic urethane resins. Of these, epoxy resins, thermosetting urethane resins, thermoplastic urethane resins, and acrylate (co)polymer resins are preferred, with the thermoplastic urethane resins being most appropriate.

Preferably the adhesive layer has a gage of 0.1 to 30  $\mu\text{m}$ , more preferably 0.2 to 25  $\mu\text{m}$ , and even more preferably 0.3 to 20  $\mu\text{m}$ .

It is recommended that the solid golf ball thus constructed have spin consistency between the dry state and the wet state. Provided that the ball receives a spin rate  $S1$  (rpm) in the dry state when hit with a short iron having a loft of an 8-iron or greater and the ball receives a spin rate  $S2$  (rpm) in the wet state when hit with the same short iron, the percent spin retention given by  $(S2/S1) \times 100$  is preferably at least 47%, more preferably at least 48%, even more preferably at

least 49%, further preferably at least 50%, and most preferably at least 51%. If the percent spin retention  $[(S2/S1) \times 100]$  is less than 47%, the difference in spin rate between the dry state and the wet state may be too large to accomplish the desired consistent spin control effect and lead to noticeable variations in flight distance or carry, failing to achieve the objects and advantages of the invention. As noted in the preamble, the "dry state" refers to the state of a golf course in normal conditions such as in fine weather, and the "wet state" refers to the state of a golf course in rain weather or when the lawn is dewed, specifically the state that the golf ball surface is wetted with water.

The multi-piece solid golf ball of the invention is a seamless golf ball on the surface of which a multiplicity of dimples are substantially uniformly arranged so that a great circle which does not intersect with the dimples is absent, as illustrated in FIGS. 2 to 4. The seamless feature eliminates any variation in the flight direction and distance of the ball when hit with a club which is designed to gain distance, as typified by a driver, and therefore, ensures stability.

For the arrangement of dimples, any well-known technique may be used, and no particular limit is imposed as long as the dimples are uniformly distributed. There may be employed any of the octahedral arrangement, icosahedral arrangement, and sphere division techniques of equally dividing a hemisphere into 2 to 6 regions wherein dimples are distributed in the divided regions. Fine adjustments or modifications may be made on these techniques.

The total number of dimples is generally 360 to 540, preferably at least 380, more preferably at least 390 and preferably up to 450, more preferably up to 400.

The dimples generally have a circular shape as viewed in plane. The diameter of dimples is preferably at least 1.8 mm, more preferably at least 2.4 mm, even more preferably at least 3.0 mm and preferably up to 4.6 mm, more preferably up to 4.4 mm, even more preferably up to 4.2 mm. The depth is preferably at least 0.08 mm, more preferably at least 0.1 mm, even more preferably at least 0.12 mm and preferably up to 0.22 mm, more preferably up to 0.2 mm, even more preferably up to 0.19 mm. Preferably the dimples include dimples of two or more types, more preferably three or more types, even more preferably four or more types which differ in diameter, and preferably up to six types, more preferably up to five types which differ in diameter. Dimples of different types may differ in depth as well.

Illustratively, one typical dimple arrangement on the inventive golf ball is a regular icosahedral arrangement as shown in FIG. 2 wherein 420 in total of four types of dimples D1 to D4 which differ in diameter are uniformly arranged such that there is absent a great circle which does not intersect with any dimples. Note that those dimples lying across the equator E which is one of great circles are cross-hatched in FIGS. 2, 3 and 4.

Another typical dimple arrangement on the inventive golf ball is a regular octahedral arrangement as shown in FIG. 3 wherein 392 in total of three types of dimples D1 to D3 which differ in diameter are uniformly arranged such that there is absent a great circle which does not intersect with any dimples.

In another regular icosahedral arrangement as shown in FIG. 4, 432 in total of four types of dimples D1 to D4 which differ in diameter are uniformly arranged such that there is absent a great circle which does not intersect with any dimples.

In contrast, FIG. 5 shows a pseudo icosahedral arrangement wherein 420 in total of three types of dimples D1 to D3

which differ in diameter are arranged, and no dimples lie across the equator E which is one of great circles, that is, the land continuously extends around the equator.

FIG. 6 shows another pseudo icosahedral arrangement wherein 432 in total of three types of dimples D1 to D3 which differ in diameter are arranged, and no dimples lie across the equator E which is one of great circles, that is, the land continuously extends around the equator.

FIG. 7 shows a golf ball bearing a dimple arrangement which has been applied to commercial wound golf balls. No dimples D lie across the equator E, that is, the land continuously extends around the equator.

The golf balls bearing the dimple arrangements shown in FIGS. 5 to 7, in which a great circle which does not intersect with dimples exists so that dimples are not uniformly distributed, lack flight consistency in that the balls suffer variations in the flight direction and distance when hit with a club which is designed to gain distance, as typified by a driver.

The diameter and weight of the golf ball of the invention comply with the Rules of Golf. The ball is formed to a diameter of not less than 42.67 mm and preferably up to 44 mm, more preferably up to 43.5 mm, even more preferably up to 43 mm. The weight is not greater than 45.92 g and preferably at least 44.5 g, more preferably at least 44.8 g, even more preferably at least 45 g, and most preferably at least 45.1 g.

## EXAMPLE

Examples and Comparative Examples are given below for illustrating the invention, but the invention is not limited to the following Examples.

### Examples & Comparative Examples

According to a conventional golf ball manufacturing process, two- and three-piece solid golf balls as reported in Tables 4 and 5 were prepared by forming the solid cores shown in Table 1 and successively forming thereon the cover inner and outer layers as shown in Tables 2 and 3 while forming dimples on the surface in a uniform arrangement.

TABLE 1

| Solid core composition (pbw)       |      |      |      |      |      |      |      |      |
|------------------------------------|------|------|------|------|------|------|------|------|
|                                    | ①    | ②    | ③    | ④    | ⑤    | ⑥    | ⑦    | ⑧    |
| Polybutadiene                      | 100  | 100  | 100  | 100  | 100  | 100  | 100  | 100  |
| Dicumyl peroxide                   | 1.2  | 1.2  | 1.2  | 1.2  | 1.2  | 1.2  | 1.2  | 1.2  |
| Barium sulfate                     | 12.6 | 12.3 | 13.1 | 15.1 | 21.5 | 15.2 | 20.3 | 14.9 |
| Zinc white                         | 5    | 5    | 5    | 5    | 5    | 5    | 5    | 5    |
| Antioxidant                        | 0.2  | 0.2  | 0.2  | 0.2  | 0.2  | 0.2  | 0.2  | 0.2  |
| Zinc salt of pentachlorothiophenol | 1    | 1    | 1    | 1    | 1    | 1    | 1    | 1    |
| Zinc diacrylate                    | 26   | 24   | 26   | 30   | 37   | 34   | 26   | 30   |

Note:

Polybutadiene: JSR BR11 by JSR Corp.

Dicumyl peroxide: Percumyl D by NOF Corp.

Antioxidant: Nocrack NS6 by Ouchi Shinko Kagaku K.K.

TABLE 2

| Cover<br>inner layer (pbw) | a   | b    | c  | d   | e   | f   | g |
|----------------------------|-----|------|----|-----|-----|-----|---|
| Nucrel AN4318              |     | 15   |    |     |     |     |   |
| Himilan 1706               | 50  | 42.5 |    |     |     |     |   |
| Himilan 1605               | 50  | 42.5 |    |     |     |     |   |
| Himilan 1557               |     |      |    | 50  |     |     |   |
| Himilan 1601               |     |      |    | 50  |     |     |   |
| Surlyn 9945                |     | 26   | 35 |     |     |     |   |
| Surlyn 8945                |     | 26   | 35 |     |     |     |   |
| Behenic acid               | 20  |      |    |     |     |     |   |
| Calcium hydroxide          | 3   |      |    |     |     |     |   |
| Hytrel 4701                |     |      |    | 100 |     |     |   |
| Hytrel 4047                |     |      |    |     | 100 |     |   |
| Dynaron 6100P              | 5.1 | 2    | 48 | 30  | 5.1 | 5.1 |   |
| Titanium dioxide           |     |      |    |     |     |     |   |

Note that the amount of each additive is per 100 parts by weight of the resin components combined.

TABLE 3

| Cover<br>outer layer (pbw)          | A   | B   | C   | D   | E   | F   | G   |
|-------------------------------------|-----|-----|-----|-----|-----|-----|-----|
| Hytrel 4701                         |     |     | 100 |     |     |     |     |
| Pandex TR3080                       | 30  | 20  |     |     |     |     |     |
| Pandex T7295                        | 70  |     |     |     |     |     |     |
| Pandex 6098                         |     | 80  |     | 100 |     |     |     |
| Himilan 1706                        |     |     |     |     | 50  | 40  |     |
| Himilan 1605                        |     |     |     |     | 50  |     |     |
| Surlyn 7930                         |     |     |     | 37  | 22  |     |     |
| Surlyn AD8542                       |     |     |     | 40  | 24  |     |     |
| Nucrel AN4318                       |     |     |     | 23  | 14  |     |     |
| Titanium dioxide                    | 2.7 | 2.7 | 5.1 | 2.7 | 5.1 | 5.1 | 5.1 |
| Dicyclohexylmethane<br>diisocyanate | 1.5 | 1.5 |     | 1.5 |     |     |     |

Note that the amount of each additive is per 100 parts by weight of the resin components combined.

Pandex: thermoplastic polyurethane elastomers by Bayer-DIC Polymer Co., Ltd.

Nucrel: ethylene-methacrylic acid-acrylate copolymer and ethylene-methacrylic acid copolymer by Dupont-Mitsui Polymers Co., Ltd.

Himilan: ionomer resins by Dupont-Mitsui Polymers Co., Ltd.

Dynaron: hydrogenated polybutadiene by JSR Corp.

Surlyn: ionomer resins by E. I. DuPont

Hytrel: thermoplastic polyester elastomers by Toray-DuPont Co., Ltd.

Dicyclohexylmethane diisocyanate: by Bayer-Sumitomo Urethane Industry Co., Ltd.

## 12

A flight test was carried out on each of the thus prepared golf balls by the following method. Also, the spin and carry of the ball in the dry and wet states when hit with No. 9 iron (#I9) were determined, from which a percent spin retention (S2/S1×100%) and a carry difference (m) were calculated. Further, the ball was hit with a sand wedge (#SW) for approach shot to examine the spin performance and stop on the green. The results are shown in Tables 4 and 5.

### Flight test

Using a swing robot of Miyamae K.K., twenty balls of each Example were hit with a driver (#W1) at a head speed (HS) of 50 m/s. Carry and total distance were measured.

### Club used

Head: manufactured by Bridgestone Sports Co., Ltd., J's METAL, loft angle 7.5°, lie angle 57°, SUS630 stainless steel, lost wax process

Shaft: Harmotech Pro, HM-70, LK (low kick point), hardness X

### Spin

The ball was hit with No. 9 iron (#I9) at a head speed (HS) of 34 m/s, both in the dry state (humidity 40%) and in the wet state (the club face and the ball were wetted with water). The behavior of the ball immediately after impact was captured by photography, and the spin rate was calculated from image analysis.

### Approach test

Using the swing robot, ten balls of each example were hit with a sand wedge (#SW, Classical Edition by Bridgestone Sports Co., Ltd.) at a head speed (HS) of 20 m/s. The behavior of the ball immediately after impact was captured by photography, and the spin rate was calculated from image analysis. The distance over which the ball rolled to stop after landing on the green was measured.

TABLE 4

|      | Core                                            | Cover               | Example |         |        |         |
|------|-------------------------------------------------|---------------------|---------|---------|--------|---------|
|      |                                                 |                     | 1       | 2       | 3      | 4       |
|      | Type                                            |                     | ①       | ②       | ③      | ④       |
|      | Outer diameter (mm)                             |                     | 36.6    | 36.6    | 36.6   | 35.4    |
|      | Deflection under 30 kg (mm)                     |                     | 2.0     | 2.1     | 2.0    | 1.7     |
|      | Specific gravity                                |                     | 1.15    | 1.14    | 1.15   | 1.17    |
|      | inner                                           | Type                | a       | b       | c      | d       |
|      | layer                                           | Shore D hardness: A | 62      | 60      | 52     | 56      |
|      | Specific gravity                                |                     | 0.98    | 0.96    | 0.95   | 0.96    |
|      | Gage (mm)                                       |                     | 1.6     | 1.3     | 1.6    | 2.2     |
|      | Adhesive layer                                  |                     | present | present | absent | present |
|      | Cover                                           | Type                | A       | B       | C      | D       |
|      | outer                                           | Shore D hardness: B | 47      | 50      | 47     | 53      |
|      | layer                                           | Specific gravity    |         | 1.18    | 1.18   | 1.19    |
|      | Gage (mm)                                       |                     | 1.5     | 1.8     | 1.5    | 1.5     |
|      | Cover inner-outer layer hardness product: A × B |                     | 2914    | 3000    | 2444   | 2968    |
|      | Ball                                            | Weight (g)          |         | 45.3    | 45.3   | 45.3    |
|      |                                                 | Outer diameter (mm) |         | 42.7    | 42.7   | 42.7    |
|      | Dimple arrangement                              |                     | FIG. 2  | FIG. 3  | FIG. 2 | FIG. 4  |
| #W1/ | Carry (m)                                       |                     | 222.0   | 224.0   | 221.5  | 223.5   |

TABLE 4-continued

|      |                                | Example |       |       |       |
|------|--------------------------------|---------|-------|-------|-------|
|      |                                | 1       | 2     | 3     | 4     |
| HS50 | Variation (standard deviation) | 2.5     | 2.4   | 2.6   | 2.5   |
|      | Total (m)                      | 235.0   | 238.0 | 233.0 | 237.0 |
| #I9/ | Dry spin S1 (rpm)              | 8770    | 8710  | 8860  | 8680  |
| HS34 | Dry carry (m)                  | 121.0   | 122.0 | 120.5 | 122.0 |
|      | Wet spin S2 (rpm)              | 4700    | 4650  | 4780  | 4300  |
|      | Wet carry (m)                  | 129.5   | 131.0 | 129.5 | 132.0 |
|      | Spin retention S2/S1 (%)       | 54      | 53    | 54    | 50    |
|      | Carry difference (wet-dry)     | 8.5     | 9.0   | 9.0   | 10.0  |
| #SW/ | Spin (rpm)                     | 6190    | 6110  | 6230  | 5990  |
| HS20 | Stop-on-green (m)              | 6.8     | 6.9   | 6.6   | 7.2   |

TABLE 5

|                                  |                                | Comparative Example |        |        |        |         |
|----------------------------------|--------------------------------|---------------------|--------|--------|--------|---------|
|                                  |                                | 1                   | 2      | 3      | 4      | 5       |
| Core                             | Type                           | (5)                 | (6)    | (7)    | (8)    | commer- |
|                                  | Outer diameter (mm)            | 36.0                | 38.5   | 35.3   | 36.5   | cial    |
|                                  | Deflection under 30 kg (mm)    | 1.5                 | 1.4    | 2.0    | 1.7    | wound   |
|                                  | Specific gravity               | 1.22                | 1.18   | 1.19   | 1.17   | golf    |
| Cover                            | Type                           | e                   |        | f      | g      | ball    |
| inner                            | Shore D hardness: A            | 60                  |        | 47     | 40     |         |
| layer                            | Specific gravity               | 0.98                |        | 1.15   | 1.12   |         |
|                                  | Gage (mm)                      | 1.8                 |        | 1.6    | 1.6    |         |
| Adhesive layer                   |                                | absent              | absent | absent | absent |         |
| Cover                            | Type                           | E                   | E      | F      | G      |         |
| outer                            | Shore D hardness: B            | 50                  | 50     | 62     | 55     |         |
| layer                            | Specific gravity               | 0.98                | 0.98   | 0.98   | 0.98   |         |
|                                  | Gage (mm)                      | 1.6                 | 2.1    | 2.1    | 1.5    |         |
| Cover inner-outer layer hardness | product: A × B                 | 3000                | —      | 2914   | 2200   |         |
| Ball                             | Weight (g)                     | 45.3                | 45.3   | 45.3   | 45.3   |         |
|                                  | Outer diameter (mm)            | 42.7                | 42.7   | 42.7   | 42.7   |         |
| Dimple arrangement               | FIG. 5                         | FIG. 5              | FIG. 5 | FIG. 6 | FIG. 7 |         |
| #W1/                             | Carry (m)                      | 219.5               | 218.5  | 221.5  | 217.0  | 217.0   |
| HS50                             | Variation (standard deviation) | 5.1                 | 5.0    | 4.9    | 5.5    | 5.7     |
|                                  | Total (m)                      | 231.0               | 229.0  | 235.5  | 228.5  | 229.0   |
| #I9/                             | Dry spin S1 (rpm)              | 9250                | 9180   | 8310   | 8610   | 9980    |
| HS34                             | Dry carry (m)                  | 119.0               | 120.5  | 122.0  | 121.5  | 119.5   |
|                                  | Wet spin S2 (rpm)              | 4150                | 4110   | 2480   | 2930   | 4570    |
|                                  | Wet carry (m)                  | 134.0               | 134.5  | 139.0  | 138.0  | 130.0   |
|                                  | Spin retention S2/S1 (%)       | 45                  | 45     | 30     | 34     | 46      |
|                                  | Carry difference (wet-dry)     | 15.0                | 14.0   | 17.0   | 16.5   | 10.5    |
| #SW/                             | Spin (rpm)                     | 6210                | 5830   | 4400   | 5650   | 6040    |
| HS20                             | Stop-on-green (m)              | 6.6                 | 7.3    | 8.4    | 7.7    | 7.1     |

There has been described a high-quality multi-piece solid golf ball which exhibits consistent flight performance when hit with a club designed to gain distance, as typified by a driver, suppresses reduction of spin when hit in the wet state with a short iron, and offers stable ready-to-strike conditions, flight performance and spin performance under any conditions covering from the fairway (driver) to the putting green (iron).

Japanese Patent Application No. 2000-389794 is incorporated herein by reference.

Although some preferred embodiments have been described, many modifications and variations may be made thereto in the light of the above teachings. It is therefore to be understood that within the scope of the appended claims, the invention may be practiced otherwise than as specifically described.

What is claimed is:

1. A multi-piece solid golf ball comprising an elastic solid core and a resin cover enclosing the solid core, the cover being composed of a plurality of layers including an inner layer disposed adjacent to the solid core and an outer layer

disposed radially outside the inner layer, the ball being provided on its surface with a multiplicity of dimples, wherein

said solid core has a hardness corresponding to a deflection of at least 1.1 mm under an applied load of 294 N (30 kgf),

said cover inner layer has a Shore D hardness of 45 to 70, said cover outer layer has a Shore D hardness of 35 to 55, further wherein

said cover inner layer Shore D hardness is quantified as "A" and said cover outer layer Shore D hardness is quantified as "B", and A and B satisfy the relationship:  $A \times B \geq 2300$ ,

the multiplicity of dimples being substantially uniformly arranged on the ball surface such that a great circle which does not intersect with the dimples is absent, and wherein

the ball receives a spin rate S1 (rpm) in the dry state and a spin rate S2 (rpm) in the wet state when hit with a

**15**

short iron having a loft of an 8-iron or greater, the percent spin retention given by  $(S2/S1) \times 100$  is at least 47%.

2. The golf ball of claim 1 wherein said cover outer layer is softer than said cover inner layer.
3. The golf ball of claim 1 wherein said cover outer layer is formed mainly of a thermoplastic polyurethane elastomer, thermosetting polyurethane elastomer, polyester elastomer or a mixture thereof.
4. The golf ball of claim 3 wherein said cover outer layer is formed mainly of a thermoplastic polyurethane elastomer obtained using an aromatic or aliphatic diisocyanate.

5. The golf ball of claim 1 wherein said cover inner layer is formed mainly of an ionomer resin.

6. The golf ball of claim 1, further comprising an adhesive layer between the cover inner and outer layers.

7. The golf ball of claim 1 wherein said core has a specific gravity of 1.0 to 1.3, said cover inner layer has a specific gravity of 0.8 to 1.4, and said cover outer layer has a specific gravity of 0.9 to 1.3.

8. The golf ball of claim 1 wherein the dimples have a circular shape as viewed in plane and have a diameter and a depth of 1.8 to 4.6 mm and of 0.08 to 0.22 mm, respectively.

9. The golf ball of claim 7 wherein the dimples include 25 dimples of three to six types which differ in diameter and/or depth.

10. The golf ball of claim 7 wherein the total number of dimples is 360 to 540.

11. A multi-piece solid golf ball comprising an elastic 30 solid core and a resin cover enclosing the solid core, the cover being composed of a plurality of layers including an inner layer disposed adjacent to the solid core and an outer layer disposed radially outside the inner layer, the ball being provided on its surface with a multiplicity of dimples, 35 wherein

said solid core has a hardness corresponding to a deflection of at least 1.1 mm under an applied load of 294 N (30 kgf),

said cover inner layer has a Shore D hardness of 45 to 70,

**16**

said cover outer layer being formed mainly of a thermoplastic polyurethane elastomer obtained using an aromatic diisocyanate and has a Shore D hardness of 35 to 55, and

the multiplicity of dimples are substantially uniformly arranged on the ball surface such that a great circle which does not intersect with the dimples is absent, the ball receiving a spin rate S1 (rpm) in the dry state and a spin rate S2 (rpm) in the wet state when hit with a short iron having a loft of an 8-iron or greater, the percent spin retention given by  $(S2/S1) \times 100$  is at least 47%.

12. The golf ball of claim 11 wherein said cover outer layer is softer than said cover inner layer.

13. A multi-piece solid golf ball comprising an elastic solid core and a resin cover enclosing the solid core, the cover being composed of a plurality of layers including an inner layer disposed adjacent to the solid core and an outer layer disposed radially outside the inner layer, the ball being provided on its surface with a multiplicity of dimples, wherein

said solid core has a hardness corresponding to a deflection of at least 1.1 mm under an applied load of 294 N (30 kgf),

said cover inner layer has a Shore D hardness of 45 to 70, said cover outer layer being formed mainly of the reaction product of a thermoplastic polyurethane elastomer with an isocyanate compound and has a Shore D hardness of 35 to 55, and

the multiplicity of dimples are substantially uniformly arranged on the ball surface such that a great circle which does not intersect with the dimples is absent, and provided that the ball receives a spin rate S1 (rpm) in the dry state and a spin rate S2 (rpm) in the wet state when hit with a short iron having a loft of an 8-iron or greater, the percent spin retention given by  $(S2/S1) \times 100$  is at least 47%.

14. The golf ball of claim 13 wherein said cover outer layer is softer than said cover inner layer.

\* \* \* \* \*